

Patented May 6, 1924.

1,492,973

# UNITED STATES PATENT OFFICE.

CHARLES T. EVANS, OF TITUSVILLE, PENNSYLVANIA, ASSIGNOR TO CYCLOPS STEEL COMPANY, OF NEW YORK, N. Y., A CORPORATION OF NEW YORK.

## STEEL ALLOY.

No Drawing.

Application filed December 4, 1920. Serial No. 428,205.

To all whom it may concern:

Be it known that I, CHARLES T. EVANS, a citizen of the United States, residing at Titusville, county of Crawford, and State of Pennsylvania, have invented certain new and useful Improvements in Steel Alloys, fully described and represented in the following specification.

This invention relates to improvements in steel alloys, and has for its object to produce a steel of the nickel-chromium type which possesses hardness, toughness, high resistance to corrosion, and which further has the property of being hardened by the ordinary heat treatment, that is, by heating and quenching in a usual quenching medium, such as water or oil.

Many steels of the so-called nickel-chromium type possess great advantages for many purposes, but they are subject to marked limitations in use. When the alloys have certain nickel, chromium and carbon contents typical of nickel-chromium steels, the resulting steels are so hard that they cannot be machined. Articles made from such steels, therefore, which require to be put into special form, must be forged, which is expensive. If, on the other hand, the proportions of nickel, chromium and carbon be such that the steel can be machined, the resulting machined articles cannot be hardened by ordinary heat treatment, that is, by subjecting them to heat and hardening in a quenching medium, such as water or oil. For instance, a typical chromium-nickel steel has a nickel content of about 3.5%, chromium, 1.5%, manganese, 0.45%, and carbon, 0.2. This steel can be machined, but the machined article cannot be hardened by the ordinary heat treatment. Case hardening can, of course, be resorted to, but this is objectionable in many instances. Again, a steel having a nickel content of 3.5, chromium 1.25, carbon 0.4, manganese 0.4%, nickel 3.5%, exhibits a scleroscopic hardness of 76. Such a steel can scarcely be touched by a file, and, of course, cannot be machined.

In general, it may be said, increasing the percentages either of carbon or of chromium, or both, will increase the hardness of the alloy and thus render it difficult, if not impossible to machine. Increasing the percentage of nickel in the alloy tends to reduce the scleroscopic hardness, but if the

nickel is added in sufficient quantity to effect such reduction in hardness as to bring the steel within machining limits, it cannot be hardened by ordinary heat treatment.

Steels which might be said to be of the nickel-chromium type have been produced for certain special purposes, such, for instance, as jewelers' die work. Such steels are relatively high in carbon and relatively low in nickel and chromium, the nickel being about, say, 1.40%, and the chromium, say, about 0.65%. Such steels can be hardened by ordinary heat treatment, but they lack the valuable characteristics imparted to the steel by higher percentages of chromium and nickel and their range of usefulness is accordingly limited.

I have found by the addition to steel alloys of the nickel-chromium type, of refractory metals of the carbon group, say, for instance, zirconium or titanium, or both, and silicon, where the silicon in the alloy is not above normal, that is, about 0.15% to 0.2%, steels can be produced in which the percentages of chromium, or chrome and nickel, are relatively high and yet the steel articles produced therefrom can be machined and subsequently hardened by the ordinary heat treatment, namely, heating and quenching in a usual medium, such as water or oil.

The amounts of refractory metal, such as zirconium or titanium and silicon added, will depend on varying conditions, such as the percentages of the other constituents of the alloy and the use to which the articles are to be put. I have found that where the combined percentage of nickel and chromium amounts to about 15%, the nickel being about 7% and the chromium 8%, satisfactory results were obtained by adding 3½% of silicon, zirconium and titanium. In the case referred to, the silicon added amounted to about 2½%, the zirconium 0.5%, and the titanium 0.25%. In the particular instance referred to, the silicon content of the alloy, prior to the addition of the refractory metals, was about normal, that is, about 0.15% to 0.2%. In this case, the scleroscopic hardness, after heat treatment and quenching was about 75 to 80.

In another instance, where the combined percentage of chromium and nickel was 12%, the nickel being 6%, and the chromium

6%, satisfactory results were obtained by adding 5.8% of the refractory metals, the silicon being 4%, zirconium 1.05% and the titanium 0.75%. In this case, the silicon content of the alloy, before the addition of the silicon, was, as before, normal. In this case, the sclerostopic hardness was slightly less than the case given before, that is, it was 65 to 70. Specific rules for the addition of the refractory metals of the carbon group cannot be given as the amounts to be added will, as before indicated, depend on the amount of hardness it is desired to produce and on the percentages of the other constituents of the alloy. In general, it may be said that if the chromium content of the alloy is lowered, the percentage of silicon added should be increased and vice versa, and if the nickel content of the alloy be lowered, the zirconium and titanium content should be increased, and vice versa. Of course, if the silicon content of the alloy, prior to the addition of the refractory metals, be either above or below the normal, the amount of silicon added will be varied to compensate for this variation.

As has been indicated, by the addition of refractory metals of the carbon group to nickel-chromium alloys, steels can be produced which can be machined and which after machining, can be hardened by ordinary heat treatment, i. e., heating and quenching in a usual quenching medium, such as water or oil. Such steels, of course, present many advantages for many uses. Such steels, furthermore, have the further advantage of being highly non-corrosive, that is, they are not attacked by vegetable acids and they are not subject to atmospheric corrosion.

What is claimed is:

1. A steel comprising carbon, manganese, nickel, chromium and iron, and also containing silicon above 0.2%, and at least one refractory metal of the carbon group, the proportions of carbon, nickel, chromium, manganese, silicon and iron being such that the steel, prior to the addition of the refractory metal, cannot be hardened by heat treatment and quenching, and the proportions of refractory metal added being such that the resulting steel can be hardened by heat treatment and quenching. 45 50

2. A steel comprising carbon, manganese, nickel, chromium and iron, and also containing silicon above 0.2% and zirconium, the proportions of carbon, nickel, chromium, manganese, silicon and iron being such that the steel, prior to the addition of the silicon and zirconium, cannot be hardened by heat treatment and quenching, and the proportions of silicon and zirconium added being such that the resulting steel can be hardened by heat treatment and quenching. 55 60

3. A steel comprising carbon, manganese, nickel, chromium and iron, and also containing silicon above 0.2% and zirconium and titanium, the proportions of carbon, nickel, chromium, manganese, silicon and iron being such that the steel, prior to the addition of the silicon and zirconium, cannot be hardened by heat treatment and quenching, and the proportions of silicon, zirconium and titanium, added being such that the resulting steel can be hardened by heat treatment and quenching. 65 70 75

In testimony whereof, I have hereunto set my hand.

CHARLES T. EVANS.